

F. W. STOCKTON,  
METHOD OF PURIFYING COTTON SEED HULL FIBER.  
APPLICATION FILED JUNE 13, 1917.

1,295,078.

Patented Feb. 18, 1919.

Fig. 1,



Fig. 2



F. W. Stockton Inventor  
By his Attorneys  
Pearce Davis Marvin & Edmonds

# UNITED STATES PATENT OFFICE.

FRANK W. STOCKTON, OF PITTSBURGH, PENNSYLVANIA, ASSIGNOR TO EAST ST. LOUIS COTTON OIL COMPANY, OF NATIONAL STOCK YARDS, ILLINOIS, A CORPORATION OF ILLINOIS.

## METHOD OF PURIFYING COTTON-SEED-HULL FIBER.

1,295,078.

Specification of Letters Patent. Patented Feb. 18, 1919.

Application filed September 13, 1917. Serial No. 191,246.

To all whom it may concern:

Be it known that I, FRANK W. STOCKTON, a citizen of the United States, residing at Pittsburgh, in the county of Allegheny, 5 State of Pennsylvania, have invented certain new and useful Improvements in Methods of Purifying Cotton-Seed-Hull Fiber; and I do hereby declare the following to be a full, clear, and exact description of the invention, 10 such as will enable others skilled in the art to which it appertains to make and use the same.

This invention relates to the purifying of cotton-seed hull fiber, and includes a novel 15 method of purifying such fiber.

After the cotton is removed from the cottonseed by ginning, most of the remaining shorter fibers are removed by what is known as the delinting operation, somewhat similar to that of ginning, the shorter fiber thus removed in the delinting process being called "linters". After the delinting process there nevertheless remains on the cottonseed a small amount of a kind of fiber or 25 fuzz which is not removed by the delinting process and which is usually made up of immature cotton fiber, averaging about three-sixteenths of an inch in length. In order to obtain this short fiber from the 30 seeds, the hulls are separated from the meats, as by the usual hulling or decorticating process, and the separated hulls are passed through an attrition mill consisting essentially of two steel disks facing and al- 35 most touching each other and running in opposite directions and having grooves in their faces. When the cottonseed hulls are fed through the center of one of these disks to the narrow space between the disks, they 40 are subjected to high speed attrition and the fiber is thereby cut off from the hulls and the hulls incidentally ground up. The fiber and ground hulls escape from the periphery of the disks and are discharged to 45 a separator, which separates the fiber from the ground hull.

The cottonseed hull fiber thus obtained contains usually about twenty-five per cent. of the cottonseed hull in the form of fine 50 particles or flakes, and with practically all the fibers attached to these fine flakes.

The present invention relates to the purification of the crude fiber thus admixed with and attached to the fine scales or par-

ticles; and has for its primary object the 55 purification of such fiber and the separation and removal therefrom of the scales and hull particles.

The purification process of my invention comprises a boiling of the impure fiber and 60 associated hull particles in dilute alkaline liquor to soften the hull particles so that they may be more readily disintegrated, or otherwise softening the hull particles; after 65 which the impure fiber thus treated is subjected to a rolling operation to disintegrate and mash the softened hull particles; and the fiber is then separated from the disintegrated and separated hull particles by a 70 special washing operation.

In the carrying out of the first step of the process, I have found it of advantage to boil the fiber in alkaline water containing, for example, about four per cent. of caustic 75 soda for about five hours. Such alkaline liquor has no injurious effect upon the fibers themselves, but it attacks the hull particles more especially and softens them so that they can be disintegrated.

This softening of the hull particles may 80 also be accomplished by suitable treatment with solutions of substances other than alkalies and even with water alone. The boiling operation may be conducted under pressure, as in an autoclave. The softening may 85 also be effected by fermentation or by enzym action.

After the fibers and their associated hull particles have been treated, and the hull particles have been thus softened, the material is passed several times between powerful steel rolls for the purpose of mashing the hull particles without seriously mashing the fiber. Inasmuch as the hull particles are 90 much thicker than the fiber, and also are softer, it is easy to effect this mashing operation, by proper adjustment of the rolls, without serious injury to the fiber. By this rolling operation most of the fiber is detached from the hull particles, and the hull 95 particles are extremely finely disintegrated. This disintegration may extend, to some extent, even to the ultimate constituent cells.

After the mashing operation, the mashed 100 mass of fiber and hull is treated for the removal of the very fine particles of hull from the fiber. I have found it of particular advantage to effect this removal in the appa-

ratus illustrated, more or less conventionally and diagrammatically, in the accompanying drawing; in which:

Figure 1 is a top view of the apparatus 5 with parts removed; and

Fig. 2 is a vertical longitudinal section on the line 2—2 of Fig. 1.

The apparatus illustrated is made up of the tank 1, containing water maintained at 10 a suitable level indicated at 2. The tank has a central division wall 3, spaced away from the ends of the tank to permit free flow of the liquor therebetween. Within the tank, on one side of the central partition, 15 is a drum or wheel 6, having longitudinal teeth thereon. This drum is arranged above an elevated portion 4 of the tank which has corresponding or complementary teeth 5, between which and the teeth on the drum 6 the 20 liquor and contents of the tank are circulated and agitated. The arrangement of these teeth is also such that they beat up and separate the fiber and fine hull particles and form them into a suspension in the water 25 contained in the tank. The drum 6 may be driven in any suitable manner, as by the pulley 7.

On the opposite side of the central partition, and near the other end of the tank, is 30 a revolving screen 8, suitably mounted and supported and driven by means of the pulley 9. The bearing at the end of this screen is hollow as indicated at 10, and has extending therethrough the outlet pipe 11 and the 35 inlet pipe 13. The pipe 11 has its inner end extending downwardly at 12 and has its outer end connected to a pump, (not shown), for pumping the water from the tank after it has passed through the screen. The pipe 40 13 terminates in a series of spray nozzles indicated at 14, and arranged to spray water through the screen from the inside and thereby remove adhering particles from the outside of the screen. The spray nozzles 45 are arranged above the level of the water in the tank so that the material removed thereby will flow back in the tank. Suitable guards 15 and 16 are shown covering the rotary screen and the rotary drum, respectively.

In the operation of the apparatus described, the mashed fiber and associated hull particles are put into the machine which is filled with water to the proper level. As 55 the material passes between the drum 6 and the bottom of the tank, it is beaten up and the fibers and fine hull particles are separated from each other and the finely divided material is thereby maintained in suspension, the circulation taking place in the direction indicated by the arrows. When 60 the rotary screen, which is of wire gauze having about 60 mesh to the linear inch, is started in operation and rotated slowly, and 65 the water spray 14 and pump for removing

the water through the pipe 11 are in operation, the water will be drawn through the screen and will be removed from within the screen through the pipe 11, carrying with it the fine suspended hull particles, 70 which are of a fineness permitting them freely to pass through the screen. The fiber, because of its length, is held on the outside of the screen and is washed off by the spray 14 and returned to the tank. In practice, 75 the rotary screen is revolved slowly, while the rotary drum 6 is rotated at high speed to give the desired agitation and beating up and separation of the fiber and hull particles. 80

By continuing the operation in the manner described for a sufficient period of time, for example, for an hour and a half, the fiber can be substantially freed from the hull particles. I have found that it is easy 85 in this way to treat cottonseed hull fiber originally containing about twenty-five per cent. of hull particles and to reduce the amount of such particles to about one per cent. or even less. At the end of the purification process, the purified fiber is removed from the tank, as by a draw-off opening (not shown) and separated from the accompanying water by filtration, or transferred to a space of storage for further treatment. 90 Where dry fiber is desired, the water can be removed by filtering and by drying, as will be readily understood.

The fiber thus purified can be subjected to a further purification process, if necessary or desirable, and, because of the substantially complete removal of the hull particles, any remaining purification can be readily made by well known methods. This final purification will depend upon the use 100 to which the fiber is to be put; and may consist of a further boiling with lye, followed by bleaching with chlorin or hypochlorite. Also, the fiber may be treated with benzine or other suitable solvent, to remove the fatty 110 or waxy matter, etc.; or this extraction process may take place in conjunction with other purification processes or before or after such other treatment. The improved process of my invention makes unnecessary 115 any elaborate subsequent purification and gives a product which can readily be treated, after a further final purification where this is necessary, for nitrating or other purposes.

The process of the present invention is 120 not intended for the treatment of crushed cottonseed hulls for the preliminary separation of the hull and fiber. Such a preliminary separation of the hull and fiber is usually effected after the crushed hulls have 125 been passed through an attrition mill, as hereinbefore described. The process of the present invention is intended for the purification of the crude cottonseed hull fiber obtained as a result of such a preliminary sep- 130

aration of the hull and fiber, as herein described. By the expression "cottonseed hull fiber" in the appended claims is therefore meant the crude fiber obtained from the 5 crushed cottonseed hulls, and containing about twenty-five per cent. of the cottonseed hull. This crude "cottonseed hull fiber" is thus principally composed of cotton fiber, and such hull as it contains is in the form 10 of fine particles or flakes.

I claim:—

1. The method of purifying cottonseed hull fiber and of separating the fiber from associated hull particles, which comprises 15 softening the hull particles, mashing the material to disintegrate the softened hull particles and detach the fiber therefrom, and subjecting the mashed material to a cleaning 20 operation and thereby washing the fine hull particles from the fiber, substantially as described.

2. The method of purifying cottonseed hull fiber and of separating the fiber from associated hull particles, which comprises 25 softening the hull particles by treatment with dilute alkaline liquor, mashing the material to disintegrate the softened hull particles and detach the fiber therefrom, and subjecting the mashed material to a cleaning 30 operation and thereby washing the fine hull particles from the fiber, substantially as described.

3. The method of purifying cottonseed hull fiber and of separating the fiber from associated hull particles, which comprises 35 softening the hull particles, passing the material between rollers and thereby mashing and disintegrating the hull particles and separating the fiber therefrom, and subjecting the mashed material to a cleaning operation and thereby washing the fine hull particles from the fiber, substantially as described.

4. The method of purifying cottonseed

hull fiber and of separating the fiber from 45 associated hull particles, which comprises softening the hull particles, mashing the material to disintegrate the softened hull particles and detach the fiber therefrom, subjecting the resulting material, in admixture 50 with water, to a beating operation to complete the separation of the fiber and hull particles and to form a suspension thereof in the water, and filtering off the water and fine hull particles from the fiber, substantially 55 as described.

5. The method of purifying cottonseed hull fiber and of separating the softened hull particles therefrom, which comprises mashing the material to disintegrate the hull particles and separate the fiber therefrom, subjecting the resulting material, in admixture 60 with water, to a beating operation and thereby separating the fiber and hull particles and forming a suspension thereof in the water, 65 subjecting the suspension to a progressive filtering operation and thereby filtering and removing the water and finely suspended particles of hull from the fiber, adding fresh amounts of water and continuing the beating 70 and filtering operation until the fiber has been purified from the hull particles, substantially as described.

6. The method of purifying cottonseed hull fiber and of separating the hull particles therefrom, which comprises boiling 75 the fiber in alkaline water containing about four per cent. of caustic alkali for about five hours to soften the hull particles, passing the boiled fiber between rolls and thereby mashing and disintegrating the hull particles, and subjecting the mashed material to a cleaning operation and thereby separating the fine, disintegrated hull particles from the fiber, substantially as described. 80 85

In testimony whereof I affix my signature.

FRANK W. STOCKTON.